

## 1

3,573,111

### HIGH LUBRICITY CORROSION RESISTANT THREADED FASTENER AND METHOD

Raymond L. Thurston, Dearborn, Mich., assignor to  
Microdot Inc., Greenwich, Conn.

No Drawing. Filed Sept. 6, 1968, Ser. No. 774,555

Int. Cl. C23f 7/10

U.S. CL. 148—6.15

8 Claims

#### ABSTRACT OF THE DISCLOSURE

A method of preparing a high lubricity corrosion resistant threaded fastener or other coated substrate product comprising the steps of: (a) cleaning the substrate, for example in a soap bath, (b) water rinsing, (c) applying an aqueous acidic metallic phosphate coating solution to the substrate, (d) applying a corrosion resistant oil to the substrate, and (e) applying a mixture of solid lubricant particle dispersion and water soluble corrosion resistant oil to the substrate; and, the coated product formed by the above method.

#### BACKGROUND OF THE INVENTION

This invention broadly relates to a surface treatment for various substrate products wherein it is desired to impart to the substrate high lubricity and corrosion resistance, and for certain applications the surface is also provided with highly desirable break-in allowance properties. The substrate products referred to are various types of fasteners such as threaded fasteners, slide mechanisms, bearings, or various mechanical components which are subjected to engine break-in wear. All of such substrates can be subjected to the surface treatment of this invention as disclosed hereinafter.

In the past, cadmium plating has frequently been used for fastener surface treatment in order to provide the fastener surface with corrosion resistance; and, also the cadmium plated fastener surface has in the past been treated with wax to provide the cadmium plated fastener with high lubricity as well as corrosion resistance. The cadmium-wax fastener surfaces which have been so treated are generally bright and silvery white in their appearance. The corrosion resistance of such cadmium-wax treated fasteners is very good particularly when a supplemental chromate treatment of the fastener surface is made. Salt spray test results (ASTM test B-117-61) on such cadmium treated fasteners result in 96 hour plus salt spray exposure times. These cadmium treated fasteners also have been found to have a hardness greater than that of the substrate base material of the fastener. However, there has been a distinct and definite problem with the cadmium-wax treated fasteners and this problem has been one of an inordinately high cost of producing same. Accordingly, there has been a long felt need in the art to develop a surface treated product or method of producing same which would exhibit comparable or better corrosion resistance, and also comparable or better lubricity as compared to a cadmium-wax surface treated substrate product, while at the same time said sought-after product had to be feasible of commercial production and economical and readily capable of being produced.

Accordingly, it is a primary object of this invention to provide an improved surface treated product which possesses high lubricity and corrosion resistance.

## 2

Another object of the present invention is to provide a highly lubricating composition which when applied in the surface treatment of a substrate fastener product would greatly improve the lubricity of the fastener, for example, a prevailing torque type fastener, while at the same time providing said fastener with maximum corrosion resistance.

Another object of the present invention is to provide an improved fastener product with the surface thereof possessing high lubricity and high corrosion resistance.

Another object of the present invention is to provide a method of preparing said improved fastener product.

Still another object of the present invention is to provide an improved coated substrate product, with the surface thereof possessing properties of high lubricity, corrosion resistance, and a surface which possesses desirable break-in allowance properties; and, the method of preparing said improved coated substrate product.

Other objects, features and advantages of the present invention will become apparent from the subsequent description and the appended claims.

#### SUMMARY OF THE INVENTION

25 The above and related objects, generally stated, are accomplished in conjunction with the solution of the problem underlying this invention by the discovery that a substrate product may be surface treated with a metallic phosphate coating to provide corrosion resistance then subsequently treated with a corrosion resistant oil to enhance the corrosion resistance, and then finally treated with a mixture of a lubricant particle dispersion and corrosion resistant oil to thereby provide the surface with unique properties of high lubricity in combination with high corrosion resistance.

30 35 The details of this invention will be more specifically described hereinafter.

Briefly stated, this invention comprises a method of preparing a high lubricity, corrosion resistant, fastener or other coated substrate product comprising the steps of: 40 cleaning the substrate, applying an aqueous acidic metallic phosphate coating solution to the substrate, applying a corrosion resistant oil to the substrate, and applying a mixture of solid lubricant particle dispersion and water soluble corrosion resistant oil to the substrate, said lubricant being selected from the group consisting of graphite, molybdenum disulfide, or vermiculite, said lubricant particle size being from about 0.5 to about 200 microns, said dispersion containing between about 2% and about 50 95% by weight total solids content, and said mixture containing a weight ratio of said dispersion to said oil between about 1:20 and about 20:1. From a product aspect this invention comprises a coated substrate product prepared in accordance with the method stated above.

#### DESCRIPTION OF THE PREFERRED EMBODIMENTS

While the exact theory of operation which underlies the invention is not exactly understood, and while it is not intended to limit the scope or application of the invention by reliance on any particular theory of operation, it is believed that the phosphate coating which is applied to the substrate surface after application leaves small pores or openings in the phosphate coating or crystal structure which allow for absorption or receipt of the corrosion resistant oil which is subsequently applied thereto. Normally in the prior art after a phosphate coating has

been applied, a sealing after-treatment is applied thereto generally comprised of a chromic acid or mixed chromic and phosphoric acid rinse. However, in the present invention no such chromic acid or phosphoric acid sealing after-treatment is applied, rather and simply a corrosion resistant oil is first applied to the phosphate coated surface and it is believed that this corrosion resistant oil is absorbed or received into the porous openings or crystalline openings of the phosphate coated surface without sealing off same. If the normal sealing after-treatment were applied subsequent to the phosphate coating, then porous openings or the like, would be closed up. However, by first applying the corrosion resistant oil which is absorbed into the porous openings the corrosion resistance of the phosphate coating is enhanced. Furthermore, by subsequently applying a mixture (disclosed hereinafter) of a lubricant particle dispersion and water soluble corrosion resistant oil to the oil treated surface, it has been discovered that this application of the mixture of lubricant particles and corrosion resistant oil is still absorbed, or received into small openings or pores in the phosphate coating, to thereby impart to the phosphate coated surface a high lubricity coating which is also at the same time highly corrosion resistant. Still further, it has been found that if only a lubricant particle dispersion is used as the last coating application to the substrate that then a satisfactory product is not obtained for the reason that the lubricant particle dispersion alone will not penetrate or leave a high lubricity surface finish on the substrate without the presence of the corrosion resistant oil.

The cleaning of the substrate surface to carry out the method disclosed herein may be carried out in any conventional manner and for example, the cleaning of the substrate surface may be carried out by immersing the substrate in a soap bath for a sufficient period of time and then cold water rinsing the substrate. Those skilled in the art will realize that there are numerous different ways of properly cleaning the substrate such that it is ready for use in the method disclosed herein.

The metallic phosphate coating solution which is selected for use in the method of this invention may satisfactorily be any aqueous acidic metallic phosphate solution which is known to form a protective phosphate coating on metallic surfaces and this includes coating solutions of zinc phosphate, manganese phosphate, iron phosphate, or the like. Preferably, the phosphate coating solution which is applied should be of the zinc phosphate type.

Examples of typically suitable phosphate coating solutions for use herein are set forth below numbered as Examples 1, 2, 3, 4 and 5:

#### EXAMPLE 1

For the aqueous acidic metallic phosphate coating solution, the following solution would be used containing: 1 1/4 pounds zinc phosphate, 3 1/4 pounds  $H_3PO_4$ , 3/4 pound of  $HNO_3$ , 1/4 ounce of  $Ni(NO_3)_2$ , and the balance water to make 100 pounds of solution.

This phosphate solution would be satisfactory for use at a temperature of approximately 90° F.

#### EXAMPLE 2

A metallic phosphate coating solution containing the following materials would be used: 22 grams per liter  $P_2O_5$ , 35 grams per liter  $NO_3$ , and 19.5 grams per liter zinc.

#### EXAMPLE 3

Aqueous acidic metallic phosphate coating solution would be used containing as follows: 11.5 grams per liter zinc, 14 grams per liter  $NO_3$ , and 13 grams per liter  $P_2O_5$ .

#### EXAMPLE 4

Aqueous acidic metallic phosphate coating solution would be used containing as follows: 10 grams per liter  $P_2O_5$ , 27 grams per liter zinc, 6 grams per liter  $ClO_3$ .

#### EXAMPLE 5

An aqueous acidic manganese phosphate coating solution would be used containing as follows:

|    |                             | Weight-grams              |
|----|-----------------------------|---------------------------|
| 5  | $Mn(H_2PO_4)_2 \cdot 2H_2O$ | 80.00                     |
|    | $HNO_3$ (42° Baumé)         | 3.00                      |
|    | $NaNO_3$                    | 10.90                     |
|    | $NaHF_2$                    | 0.90                      |
| 10 | $K_2TiF_6$                  | 2.10                      |
|    | Water                       | 94.9                      |
|    | Total                       | <sup>1</sup> 191.8        |
|    |                             | <sup>1</sup> 133 ml. vol. |

15 A particularly preferred phosphate coating solution would be an aqueous zinc-iron phosphate solution such as Phosphotex A-8 available from the MacDermid Chemical Company of Waterbury, Conn. Phosphotex A-8 contains an acid ratio between 5 and 7, that is, a ratio determined from the total acid divided by the free acid; and, a ferrous iron content of 0.1 to about 0.7% by weight; and, a zinc content of 0.20% by weight minimum.

20 The time period of application for the phosphate coating solution should broadly be within the range of about  $\frac{1}{2}$  up to 120 minutes. Preferably this time period should be within the range of from about 5 minutes up to about 60 minutes, and most suitable results are obtained when the time period is within the range of about 15 minutes up to about 45 minutes.

25 30 The application temperature or dipping temperature for the phosphate coating solution should be within about the range of about 50° up to about 220° F. and preferably the dipping temperature range should be from about 100° up to about 210° F. Most suitable results are obtained when this temperature range is from about 180° F. up to about 200° F.

35 The corrosion resistant oil which is applied to the substrate after the phosphate coating solution has been applied may be described as follows. First, any number of 40 different corrosion resistant oils may be used for application to the substrate subsequent to the application of the phosphate solution, and those skilled in the art will be aware of numerous different corrosion resistant oils which may be used for this purpose. Preferably this corrosion 45 resistant oil would be of the conventional type which are known to be either dispersible or emulsifiable in water, that is, a water soluble corrosion resistant oil. This corrosion resistant oil should be one which is capable of being used over a phosphate coating to produce a generally dry 50 to the touch corrosion resistant film. A particularly suitable corrosion resistant oil for this purpose is the trademark oil Metex-M-685, available from the MacDermid Chemical Company. Metex 685 oil is used at a 10-20% by volume amount in water and is applied from an oil 55 bath at an operating temperature most suitably within the range of about 115°-145° F. The application time period for this corrosion resistant oil should most specifically be at an immersion time period of about 30 seconds or longer. Another suitable oil is Northwest Seal Oil 60 available from Northwest Chemical Company.

65 Suitable corrosion resistant oils may more specifically be described as those oils comprising a mixture of paraffin oil, oxygenated paraffin oils, and a carbitol solvent.

The application time or immersion time in the corrosion 70 resistant oil should broadly be from about  $\frac{1}{20}$  of a minute up to as long as is convenient. Preferably, the application time for the corrosion resistant oil should be within the range of about  $\frac{1}{2}$  up to about 120 minutes and most suitably the application time period is within the range of about  $\frac{1}{2}$  up to about 60 minutes.

The application temperature or the immersion temperature of the substrate in the corrosion resistant oil should broadly be within the range of about 40° F. up to as high a temperature as is convenient, and normally this high temperature would not be more than the boiling

point temperature of the corrosion resistant oil. Preferably, the application temperature for the corrosion resistant oil should be within the range of about 85° F. up to about 200° F. and most suitably this temperature should be within the range of about 115° F. up to about 145° F.

The particular choice of the corrosion resistant oil which is applied after the phosphate coating is applied is not a critical choice<sup>1</sup> so long as the above criteria are generally met and no attempt will be made herein to exhaustively define all of the various corrosion resistant oils which could be used for the purposes of this invention.

At this point it should also be stated that after the application of the corrosion resistant oil to the substrate and the substrate is removed from application contact with said corrosion resistant oil, then a sufficient amount of time should be allowed to elapse before the substrate is taken into the next step of the method of applying a mixture of solid lubricant particle dispersion and water soluble corrosion resistant oil to the substrate. As an example, this time period which should be allowed to lapse should be approximately 10 minutes up to about 10 hours or more. Preferably, it should be from about 1/2 hour up to 8 hours. Still further, generally stated, so long as the minimum time period is allowed to lapse it is sufficient and thereafter the time period can be as high a magnitude as is desired.

There now follows a description of the step of applying a mixture of solid lubricant particle dispersion and water soluble corrosion resistant oil to the substrate.

The lubricant particle dispersion discovery in accordance with the invention herein, there should be one in which the lubricant is selected from the group consisting of graphite, molybdenum disulfide or vermiculite. Graphite is the preferred lubricant. The lubricant particles may be used either singly or in any combination thereof.

Preferably stated, the lubricant particle dispersion should be any aqueous dispersion containing a percent total of solids within the broad range of about 2% up to about 95% by weight. More specifically, the percent total solids should be within the range of about 5% up to about 80% and most suitable results are obtained using a dispersion containing from about 20% up to about 50% by weight total solids.

The lubricant particle size should broadly be within the range of about 0.5 up to about 200 microns. Higher particle sizes than 200 microns may be used for certain applications. Preferably the lubricant particle size should be within the range of about 1 up to about 100 microns. More specifically but without attempting to limit the invention, the lubricant particle size may be within the narrow range of approximately 20 microns up to about 70 microns.

As discussed hereinabove the lubricant particle dispersion used in combination with a water soluble corrosion resistant oil as a mixture thereof for application to the substrate.

The weight ratio of said dispersion to said oil should generally be within the broad range of about 1:20 to about 20:1. Preferably the weight ratio of the lubricant particle dispersion to the water soluble corrosion resistant oil should be within the range of about 1:5 to about 5:1; and, most suitably the ratio should be within the range of about 1:3 to about 3:1.

The application time period for immersion dipping or applying the mixture of lubricant particle dispersion and water soluble corrosion resistant oil to the substrate should be within the broad range of about 1/4 second up to about 2 hours. This application time may be longer for certain specific products or applications. Preferably, the application time period for the mixture should be within the range of about 1/4 second up to about one hour; and, more specifically, the application time period for the

mixture should be within the range of about 1/2 second up to about 15 minutes.

The application or the dipping temperature for applying the mixture to the substrate should broadly be within the range of about 40° F. up to about 220° F. Preferably this temperature range should be within the range of about 70 up to about 210° F. and more specifically, this temperature range should be from about 100° F. up to about 145° F.

10 The properties obtained by substrate products coated in accordance with this invention are as follows: First, products coated in accordance with this invention when tested according to the salt spray test designated ASTM test B-117-61 give values of 700 to 800 hours or higher 15 salt spray corrosion resistance results. Products coated in accordance with the invention herein possess an unexpectedly high lubricity or highly lubricated surface. This is indicated by the fact that fasteners coated in accordance with this invention have prevailing torques which 20 prevailing torques are improved by 25-50% or more at a particular given clamp load when coated in accordance with the invention herein.

In order to further illustrate the invention the following 25 additional examples are provided. It is to be understood, however, that all of the examples in this application are included for illustrative purposes and are not intended to be limiting of the scope of the invention as set forth in the subjoined claims.

#### EXAMPLE 6

30 Threaded fasteners of the prevailing torque type known to those skilled in the art were surface treated in accordance with the invention herein and rendered into a high lubricity, corrosion resistant fasteners in the following manner.

35 First, a batch of the fasteners were cleaned in a soap bath by immersion therein for approximately 5 minutes. The particular soap used for this cleaning operation was not critical and any heavy duty detergent or industrial detergent or the like may be used.

40 Second, the fasteners were subjected to a cold water rinse for approximately 30 to 60 seconds.

45 Third, the fasteners were immersed in an aqueous acidic metallic phosphate coating solution for approximately 30 minutes with the phosphate coating solution being maintained at a temperature of approximately 195° F. The coating solution used was a zinc-iron phosphate coating solution of Phosphotex A-8 as described hereinabove.

Fourth, after removal of the fasteners from the phosphate coating solution the fasteners were subjected to a hot water rinse for approximately 30 to 60 seconds at a temperature of approximately 170° F. The temperature and time period of the hot water rinse was found not to be critical.

Fifth, the fasteners were immersed in a corrosion resistant oil for a time period of approximately 1-2 minutes with the oil temperature being approximately 125-135° F. The oil used for this particular treatment was Metex-685 described hereinabove. Subsequent to the application of this oil, the fasteners were removed from the oil and allowed to stand in the open at room temperature for several hours, on a broad basis, and more specifically for about one hour.

Sixth, the fasteners were immersed in a mixture of solid lubricant particle dispersion and water soluble corrosion resistant oil for a time period of approximately 30 seconds and at an immersion temperature of approximately 130° F. The lubricant particle dispersion used was the product "Prodag" which is an aqueous dispersion of graphite in water carrier at an approximately 30% by weight solids content. The density of this specific dispersion in pounds per gallon is approximately 9.8. The product Prodag is available from Acheson Industries, Inc., Port Huron, Mich. The water soluble corrosion resistant oil used in the mixture was Metex 685 as described hereinabove. The weight ratio of the lubricant particle dispersion to the

<sup>1</sup> United States patents which disclose other suitable corrosion-resistant oils are: 2,080,299; 2,820,723; 2,861,907 and 3,215,715.

water soluble corrosion resistant oil was approximately 1:1 ratio by weight.

The fastener coated in accordance with the above description was a  $\frac{3}{8}$ -16 x  $1\frac{3}{32}$  cone lock nut of steel type 1035. This type threaded lock nut fastener when so surface treated as described hereinabove, gave a salt spray test result of 800 hours or higher. Furthermore, it was determined that the prevailing torque in inch pounds at particular clamp loads in inch pounds was improved by 25-50% or higher due to the highly improved lubricity imparted to the fastener surface, as compared to an identical fastener coated by a conventional phosphate coating process and treated with corrosion resistant oil.

#### EXAMPLE 7

The surface treatment process of Example 6 may satisfactorily be repeated except that in place of the graphite dispersion (Prodag) a dispersion is used comprised of colloidal molybdenum disulfide in water. This molybdenum disulfide dispersion has a density of 11 pounds per gallon with the molybdenum disulfide particle size being approximately 1 micron. The percent total solids of the molybdenum disulfide dispersion in the water carrier should be about 35% by weight total solids. A suitable molybdenum disulfide dispersion is Acheson Industries, Inc. product No. 206.

#### EXAMPLE 8

The process of Example 6 may satisfactorily be repeated but using instead of the graphite dispersion a dispersion of vermiculite in water at a total solids content of about 36% by weight total solids. This vermiculite dispersion has a density of approximately 11.4 pounds per gallon. The carrier for the vermiculite dispersion is water. A suitable vermiculite dispersion for use in carrying out this example would be Acheson Industries, Inc. product No. 395.

While it will be apparent that the preferred embodiments of the invention are well calculated to fulfill the objects above stated, it will be appreciated that the invention is susceptible to modification, variation and change without departing from the proper scope or fair meaning of the subjoined claims.

What is claimed is:

1. A method of preparing a high lubricity, corrosion resistant, coated fastener substrate product comprising the steps of:

cleaning the fastener substrate,  
applying an aqueous acidic metallic phosphate coating solution to the substrate,

said coating solution being selected from at least one of the group consisting of zinc phosphate, manganese phosphate, or iron phosphate coating solutions,

applying a corrosion resistant oil to the substrate, and applying a mixture of solid lubricant particle dispersion and water soluble corrosion resistant oil to the substrate,

said lubricant being selected from the group consisting of graphite, molybdenum disulfide, or vermiculite,

said lubricant particle size being from about 0.5 to about 200 microns,

5 said dispersion containing between about 2% and about 95% by weight total solids content, and said mixture containing a weight ratio of said dispersion to said oil between about 1:20 and about 20:1.

2. The method of claim 1 wherein said particle is from about 1 to about 100 microns.

3. The method of claim 1 wherein said dispersion contains between about 5% and about 80% total solids.

4. The method of claim 1 wherein said weight ratio is between about 1:5 and about 5:1.

5. The method of claim 1 wherein said particle is from about 1 to about 100 microns, said dispersion contains between about 5% and about 80% total solids,

said weight ratio is between about 1:5 and about 5:1.

6. The method of claim 1 wherein said particle is from about 1 to about 100 microns, said dispersion contains between about 20% and about 50% total solids,

said weight ratio is between about 1:3 and about 3:1.

7. The method of claim 1, 2, 3, 4, 5 or 6 wherein said lubricant is graphite.

8. A threaded fastener product comprised of a coated substrate metal having a first applied coating thereon of an aqueous acidic metallic phosphate coating solution,

of the group consisting of zinc phosphate, said coating solution being selected from at least one manganese phosphate, or iron phosphate coating solutions,

having a second applied coating thereon of a corrosion resistant oil, and

having a third applied coating thereon of a mixture of solid lubricant particle dispersion and water soluble corrosion resistant oil,

said lubricant being selected from the group consisting of graphite, molybdenum disulfide, or vermiculite,

said lubricant particle size being from about 0.5 to about 200 microns,

said dispersion containing between about 2% and about 95% by weight total solids content, and said mixture containing a weight ratio of said dispersion to said oil between about 1:20 and about 20:1.

#### References Cited

##### UNITED STATES PATENTS

|           |         |             |       |           |
|-----------|---------|-------------|-------|-----------|
| 1,964,671 | 6/1934  | Nesbitt     | ----- | 117—134X  |
| 2,266,379 | 12/1941 | Floyd       | ----- | 148—6.15X |
| 2,731,360 | 1/1956  | Love        | ----- | 148—6.15X |
| 2,899,336 | 8/1959  | Peck        | ----- | 117—134X  |
| 3,035,926 | 5/1962  | Larrieu     | ----- | 117—134X  |
| 3,297,493 | 1/1967  | Blum et al. | ----- | 117—134X  |

RALPH S. KENDALL, Primary Examiner

C. WESTON, Assistant Examiner

U.S. CL. X.R.

60 85—32, 32.1, 35

UNITED STATES PATENT OFFICE  
CERTIFICATE OF CORRECTION

Patent No. 3,573,111 Dated March 30, 1971

Inventor(s) Raymond L. Thurston

It is certified that error appears in the above-identified patent and that said Letters Patent are hereby corrected as shown below:

Column 8, line 27, "of the group consisting of zinc phosphate," should have been --said coating solution being selected from at least one--.

Column 8, line 28, "said coating solution being selected from at least one" should have been --of the group consisting of zinc phosphate, --.

Signed and sealed this 22nd day of June 1971.

(SEAL)

Attest:

EDWARD M.FLETCHER,JR.  
Attesting Officer

WILLIAM E. SCHUYLER, J  
Commissioner of Patent